# EUROPEAN PATENT APPLICATION

(11) **EP 1 925 605 A1**
(43) Date of publication of application: **28.05.2008**
(21) Application number: 07466023.4
(22) Date of filing: 21.11.2007
(51) Int. Cl.: C06B 47/00, C06B 25/18

(54) **Explosive**

(30) Priority: 23.11.2006 CZ 200618297 U
(71) Applicant: STV group A.S., 110 00 Praha 1 (CZ)
(72) Inventor: Drda, Martin, 140 000 Prah (CZ); Zapletal, Michal, 463 31 Nová Ves (CZ); Rez, Jan, 503 51 Nové Mesto (CZ)
(74) Representative: Musil, Dobroslav

(57) **Abstract**

Explosive is constituted by mixture of delaborated smokeless powder with emulsion matrix, whereas content of delaborated smokeless powder in explosive mass is 20 to 80%w/w.

## Description

### Technical Background art

In last ten years there is in Czech republic as well as in other European countries the extensive armies reduction in progress, linked with liquidation of large volumes of excessive ammunition. Liquidation generally proceeds in the form of delaboration with subsequent utilization of at least some ammunition components and /or liquidation of individual ammunition components. One of the most important delaborated ammunition components are delaborated smokeless powders. These materials are liquidated either by burning or are utilized as raw material for new smokeless powders production or are utilized at rock shooting and blasting in quarries directly as industrial explosives.
The utilization of delaborated smokeless powders at rock shooting and blasting is meaningful utilization of these materials in fact, but it brings one principal disadvantage, inhering in danger of transition of delaborated smokeless powders detonation into burning, by which strong losses of energy necessary for rock shooting and blasting happen. Delaborated smokeless powders are used for production of powdery ammonium nitrate explosive, whose disadvantage however is that they are not water resistant and therefore cannot be used in irrigated blastholes. This fact then limits the quantity of delaborated smokeless powders that is possible in such manner to use.

The aim of technical solution is to remove or at least to minimize the drawbacks of the background art

### Principle of the invention

The aim of the technical solution is reached by explosive, whose principle is that it is constituted by mixture of delaborated smokeless powder with emulsion matrix, whereas content of delaborated smokeless powder in explosive mass is 20 to 80% w/w.

The advantage of this explosive is that emulsion matrix in mixture with delaborated smokeless powder ensures necessary workability of explosive and ensures also necessary water-resistance of explosive, that all including securing of detonation reliability. Smokeless powder then contributes to augmentation of explosive sensitivity and to augmentation of explosive energetic potential.

In advantageous embodiment there is in emulsion matrix put porous granulated ammonium nitrate, coleseed oil - methylester and expanded polystyrene.

### Examples of embodiment

Explosive is constituted by mixture of delaborated smokeless powder with emulsion matrix and eventually also other additives. Emulsion matrix is withal inexplosive highly viscous substance consisting of ammonium nitrate and sodium nitrate water solution, mineral oil and emulsifier, that is sensitized by particles of delaborated powder, eventually also by glass microbeads or gas bubbles.

### Example No.1:

Explosive contains 50%w/w of emulsion matrix and 50%w/w of nitroglycerin delaborated smokeless powder.

### Example NO.2

Explosive contains 20%w/w of emulsion matrix and 80%w/w of nitrocellulose delaborated smokeless powder.

### Example No 3:

Explosive contains 80%w/w of emulsion matrix and 20%w/w of three component nitroguanidin delaborated smokeless powder.

### Example No 4:

Explosive contains 30%w/w of emulsion matrix, 40%w/w of delaborated smokeless nitroglycerin powder, 28%w/w of porous granulated ammonium nitrate, 1,5%w/w of coleseed oil-methylester and 0,5%w/w of expanded polystyrene.

## Claims

1. Explosive **characterized by** that it is constituted by mixture of delaborated smokeless powder with emulsion matrix, whereas content of delaborated smokeless powder in explosive mass is 20 to 80%w/w.

2. Explosive according to claim 1 **characterized by** that in emulsion matrix is put porous granulated ammonium nitrate, coleseed oil - methylester and expanded polystyrene.
